

W. BORCHERS & H. PEDERSEN.  
 EXTRACTION OF COPPER AND NICKEL, PARTICULARLY FROM LOW GRADE ORES AND PRODUCTS.  
 APPLICATION FILED JUNE 5, 1912.

1,101,115.

Patented June 23, 1914.



WITNESSES

E. C. Schuermann.  
 H. J. Morris.

INVENTORS

Wilhelm Borchers  
 Harald Pedersen  
 by  
 James Goldbrong & Miller  
 of Dallas.

# UNITED STATES PATENT OFFICE.

WILHELM BORCHERS, OF AACHEN, GERMANY, AND HARALD PEDERSEN, OF TRONDHJEM, NORWAY.

## EXTRACTION OF COPPER AND NICKEL, PARTICULARLY FROM LOW-GRADE ORES AND PRODUCTS.

1,101,115.

Specification of Letters Patent. Patented June 23, 1914.

Application filed June 5, 1912. Serial No. 701,859.

To all whom it may concern:

Be it known that we, Dr. WILHELM BORCHERS, professor, a subject of the German Emperor, and resident of 15 Ludwig-  
sallee, Aachen, Germany, and HARALD PE-  
DERSEN, engineer, a subject of the King of  
Norway, and resident of Trondhjem, Nor-  
way, have invented certain new and useful  
Improvements in the Extraction of Copper  
and Nickel, Particularly from Low-Grade  
Ores and Products; and we do hereby de-  
clare the following to be a full, clear, and  
exact description of the invention, such as  
will enable others skilled in the art to which  
it appertains to make and use the same.

This invention relates to the process de-  
scribed in our prior Letters Patent No.  
1,043,291 of November 5th 1912 for the ex-  
traction of nickel and copper from ores or by-  
products containing the sulfids of these  
metals together with iron and copper by a  
combination of smelting, roasting, leaching  
and precipitating operations. It has now  
been found that this process can be appre-  
ciably simplified in its latter stages.

The present improved process is carried  
out in the following manner and as dia-  
grammatically represented in the accom-  
panying drawing:

30 The first operations:—

1. Smelting the ore,
2. Roasting to sulfates,
3. Leaching with acidulated water,

4. Utilizing the leaching residue in the  
ore smelting operation, remain as described  
in the specification of the said prior pat-  
ent. The working principle of the main  
process, of first extracting the copper and  
nickel together from the ore, in a solution,  
40 thus remains as before. The succeeding  
stages are, however, varied as follows.

5. From the lye obtained from operation  
3, the copper alone is precipitated as sulfid  
by means of sulfureted hydrogen; this lat-

ter can be obtained from a portion of the 45  
crude matte by means of sulfuric acid.



6. The copper sulfid obtained in this way  
is filtered, dried and then converted by any 50  
known method into metallic copper or cop-  
per vitriol (blue vitriol), for instance by  
smelting it with copper oxid



55

or by oxidizing it



7. The nickel sulfate solution is evapo-  
rated and allowed to cool and crystallize, 60  
yielding nickel sulfate and a mother liquor,  
which latter may be utilized in the leaching  
operation 3 or returned to the roasting op-  
eration 2.

8. The nickel sulfate obtained from op-  
eration 7 is completely dried and roasted  
until it decomposes into nickel oxid, sulfuric  
acid, and sulfur trioxid, which two latter  
may be returned to the roasting operation 2.

9. The nickel oxid obtained by the op-  
eration 8 is reduced to metallic nickel by  
smelting in the known manner, viz., by re-  
duction with carbon and carbon monoxid  
in crucible-, muffle-, or electric-furnaces:



75

The simplification of the process will be-  
come even clearer on comparing the follow-  
ing tabulation with the similar summariz-  
ing of the main process. By splitting up  
the nickel sulfate into protoxid, sulfuric  
acid and sulfur trioxid, instead of precipi-  
tating it by means of sulfids as in the proc-  
ess, described in the prior patent aforesaid, 85  
the preparation of the precipitating agent  
(sodium sulfid), the addition of the lime-  
stone flux, and the formation of a waste

product (gypsum) are avoided. Acid gases are, however, evolved, which accelerate the roasting operation 2, but which, however, in-

crease the yield of sulfuric acid from this operation if it be desired to treat the waste gases for the manufacture of sulfuric acid. 5

*Synopsis of the improved process.*



Having now particularly described and ascertained the nature of our said invention and in what manner the same is to be performed, we declare that what we claim is:—

10 1. The process for extracting nickel and copper from ores and the like containing sulfids, which comprises smelting the ore to a matte, roasting the matte, leaching the

15 roasted material with acidulated water, precipitating from the resultant sulfate solution the copper by means of hydrogen sulfid, converting the precipitate into metallic copper, evaporating the residual 20 nickel sulfate solution, roasting the dried nickel sulfate to convert the same into nickel oxid, and finally reducing the same to metallic nickel.

25 2. The process of separating copper and nickel from sulfate solutions of the same, which comprises precipitating the copper from said solution with hydrogen sulfid, separating the copper sulfid and reducing the same to metallic copper, evaporating 30 the residual nickel sulfate solution, heat-

ing the residual nickel sulfate to convert the same into nickel oxid, and reducing said nickel oxid to metallic nickel.

3. The process for the extraction of nickel and copper from ores and the like containing sulfids which comprises forming from the said ores a solution of the sulfates of nickel and copper, precipitating and separating the copper as sulfid from the solution by means of sulfured hydrogen, evaporating the nickel sulfate solution, roasting the resultant nickel sulfate to convert the same into nickel oxid, and finally smelting the nickel oxid to reduce the same to metallic nickel. 45

In testimony whereof we have affixed our signatures, in presence of witnesses.

DR. WILHELM BORCHERS.  
HARALD PEDERSEN.

Witnesses:

KARL BOONEMANN,  
KARL WAGENMANN,  
JOHN SKREDDER,  
JENS JENSEN.